

## UNITED STATES PATENT OFFICE

2,266,056

## METALWORKING PROCESS

Wayne E. Martin, Temple, Pa., assignor to The Beryllium Corporation, a corporation of Delaware

No Drawing. Application July 17, 1940,  
Serial No. 345,978

7 Claims. (Cl. 148—11.5)

This invention relates to metallurgy and more particularly to metal working and has for its object the provision of a method of working cast beryllium-copper alloys containing beryllium within the range 1.5—2.10% to homogenize the structure thereof thereby to render the same better adapted for severe cold mechanical deformation and to age hardening heat treatment. Another object is to provide a method of working cast beryllium-copper alloys containing 1.5—2.10% beryllium to effect substantially complete elimination therefrom of the cast beta constituent normally present therein. Still another object is to provide a beryllium-copper alloy containing beryllium 1.5—2.10% that is substantially free from cast beta constituent, homogeneous in structure, and more readily cold workable and more uniformly age hardenable. Other objects and advantages will be apparent as the invention is more fully hereinafter disclosed.

In the manufacture of beryllium-copper alloys the same are first prepared in the molten state and then are cast into suitable sized ingots as heretofore practiced in the manufacture of other type alloys. Due to the nature of the phase diagram, in the course of freezing a marked cored structure results in beryllium-copper alloys, the precise character of which varies somewhat with respect to the rate of cooling the ingot. In general, the first nuclei to freeze are of low beryllium content (about 1%), and while the metal subsequently depositing on the nuclei becomes progressively higher in beryllium content the final metal to freeze carries about 5% beryllium. This latter constituent is known in the art as the "beta" constituent. The size or mass of this beta constituent varies widely, depending upon the rate at which the cast metal is cooled, moreover, its re-solution and redistribution of the beryllium content thereof uniformly throughout the ingot is rendered difficult by reason of the relatively low rate of diffusion of beryllium in copper, and further by the formation of zones of saturated alpha solid solution around each beta particle during solution annealing.

The cold workability and age hardening as well as the physical and mechanical properties of beryllium-copper alloys are directly effected by the presence of this beta constituent and by the uniformity of distribution of beryllium in the alloy. In general, binary beryllium-copper alloys containing less than about 1.5% beryllium are recognized as being cold workable, but not significantly age hardenable; those containing beryllium within the range 1.5 to 2.10% are recog-

nized as being both cold workable and age hardenable; and those containing over about 2.10% beryllium are recognized as being of limited cold workability depending upon the beryllium content but age hardenable and as being more suited for use as casting alloys. However, in those alloys containing beryllium within the range 1.5 to 2.10% the cold workability varies with variation in the beta content thereof and the size and distribution of the same throughout the cast ingot.

I have found that because of the relatively low rate of diffusion of beryllium in copper and the mode of formation of the same, the beta constituent in copper alloys containing 1.5—2.10% beryllium is with difficulty eliminated from the alloy and the beryllium content thereof uniformly distributed throughout the same. The following method has been found by me to be most effective in obtaining re-solution of the beta constituent and the uniform distribution of the beryllium content throughout the alloy.

I first subject the cast metal to a prolonged heating approximating three (3) hours at a temperature within the range 1400—1500° F. to obtain partial re-solution of the beta constituent. I then subject the casting to hot mechanical deformation on a falling temperature gradient, starting at temperatures approximating 1450° F., continuing the deformation until about 700° F., the extent of deformation being such as to effect partial fracture of the beta particles and a general breaking up of the surrounding alpha matrix, which during the first heating has become saturated with beryllium. Solution of the beta phase proceeds very slowly unless this saturated zone is disrupted by hot working.

I then subject the hot worked ingot to another prolonged heating approximating three (3) hours to effect further re-solution of the beta constituent and again subject the ingot to further mechanical deformation starting at 1450° F. as described above.

The beta solution heating and hot mechanical deformation operations are repeated as frequently as may be found necessary with any given alloy composition within the range 1.5—2.10% beryllium to effect re-solution of the beta constituent before the thickness of the ingot has been reduced to that at which cold mechanical deformation is to be initiated. The frequency of application of the two operations will vary with any given alloy with respect to the size of the beta particles present, and in general with any given size beta particles will increase with

increase in beryllium content within the range beryllium 1.5-2.10%. As the beryllium content approximates 1.9%, it is necessary even after cold working is initiated to subject the cold worked metal to one or more intermediate heatings at a temperature within the range 1400°-1500° F. for a prolonged time interval approximating three (3) hours to effect final re-solution of the last traces of the beta constituent, particularly if originally present in relatively large particles. Following each heating within the range 1400°-1500° F. that is applied after cold working is initiated, the alloy should be quenched or rapidly air cooled to preserve the solid solution structure obtained.

As one specific embodiment of the practice of the present invention, the working method employed on the 1.50-1.90% beryllium alloy will be described.

This alloy is usually cast as four inch (4") rounds approximating 24 inches in length. I first heat these cast ingots in a furnace under atmospheric conditions inhibiting alloy deterioration to a temperature approximating 1475° F. and maintain the ingot at this temperature for at least three (3) hours. I have found that heating for periods of time longer than three (3) hours does not appear to effect an appreciably greater amount of re-solution of the beta constituent.

I then subject the heated ingot to hot mechanical deformation, as above described, until about 35-40% reduction in area has been obtained. The hot worked metal is again soaked at about 1475° F. for another three (3) hours. Following the second heating, the metal is again hot worked to about 35-40% reduction in area and again soaked at about 1475° F.

Where the beryllium content approximates 1.50%, it will be found that the major portion of the beta constituent has been redissolved at the end of the third heating, or that a sufficient amount of the same has been redissolved to permit the metal to be mechanically deformed in the cold at least to a 50% reduction in area. Where the beryllium content approximates 1.90% and the initial particle size of the beta constituent is not excessive, it will also be found that at the end of the third heating the major portion of the beta constituent has been dissolved and that the metal can be cold worked to about 50% reduction in area.

Accordingly, at the end of the third heating I generally quench or rapidly air cool the alloy and initiate cold working on all alloys containing 1.5 to 1.90% and subject the same to about 50% reduction in area. The alloy is then given a fourth reheating within the range 1400°-1500° F. for another three (3) hour period and quenched or rapidly air cooled thereafter.

Following this heating, it will be found that the alloys are substantially free from beta constituent and are of substantially uniform composition throughout, as is reflected in the cold working properties and in the extreme uniformity in age hardening and physical properties of the alloy.

In those alloys containing between 1.90-2.10% beryllium, the re-solution of the beta constituent is more difficult by reason of the fact that the amount of beta is greater and the particle size of the same is usually larger. However, by following the practice hereinabove given with respect to the 1.5-1.90% beryllium alloys on the same sized cast ingots, modified to the extent

of increasing the total number of high temperature heatings and hot working operations by reducing the per cent reduction of area during each hot working operation and increasing the number of anneals during subsequent cold working, a final cold worked product may be obtained even with the 2.10% beryllium alloy that is substantially free from beta constituent.

For example, the 2.10% beryllium alloy in four inch (4") round casting, when subjected to substantially the same total mechanical deformation given the 1.5-1.90% Be alloy in three (3) hot working stages instead of two (2) each preceded and followed by a three (3) hour soaking at a temperature within the range 1400-1500° F., will be found to be readily cold workable to at least at 30% reduction in area if quenched or rapidly air cooled following the fourth soaking.

By then subjecting the metal to a plurality of alternate cold working and heat treating operations, each cold working operation producing a 30-40% reduction in area and each heating being a soaking for about three (3) hours at a temperature within the range 1400°-1500° F., the final cold worked metal will be found to be entirely free from beta and of uniform composition throughout. For example, I prefer to effect reduction of the four inch (4") round casting of the 2.10% Be alloy to about one inch (1") in four (4) hot working stages. After the fifth soaking heating I quench or rapidly air cool the one inch (1") hot worked material and then subject it to the following working method:

- (1) Cold work to about  $\frac{1}{2}$ ".
- (2) Anneal 3 hours at 1475° F., quench.
- (3) Cold work to about  $\frac{1}{4}$ ".
- (4) Anneal 3 hours at 1475° F., quench.
- (5) Cold work to about  $\frac{1}{8}$ ".
- (6) Anneal 3 hours at 1475° F., quench.
- (7) Cold work to desired final, or near final, size.

The product at the end of step (6) usually is completely free from beta, and can be cold worked as much as 80% reduction to desired sized wire or strip without difficulty. It is to be recognized that where material of  $\frac{1}{2}$ ",  $\frac{1}{4}$ " and  $\frac{1}{8}$ " sizes, substantially free from beta are desired, larger sized starting ingots may be employed. Alternatively, by increasing the total number of beta-solutioning heatings with interspersed hot or cold work stirring operations, it is also possible to obtain beta-free material at larger sizes.

The above disclosure relates more specifically to the so-called binary type alloy. As hereinabove disclosed, the particle size and distribution of the beta has an important bearing on the effectiveness of any given method of working followed as hereinabove described. The particle size and distribution of the beta is materially affected by the rate of cooling the casting. I have also found it to be markedly affected by alloyed percentages of one or more of the iron group metals within the range .10-.50%.

The iron group metals (Fe, Co and Ni) each appear to form beryllide compounds when present in amounts above the solubility limit of each (which in general approximates .10%). Each of these metals form a characteristic type of beryllide compound readily identifiable one from the other on microscopic examination.

These beryllide compounds appear to have a very pronounced effect on the particle size and distribution of the beta constituent in the cast alloy, causing the same to be smaller and more

uniformly distributed, probably by providing a larger number of nuclei on which crystallization may initiate. However, these beryllide compounds per se are exceedingly hard and brittle, and when present in any considerable amount above about .50% deleteriously affect the cold workability of the alloy. I have found that particularly in the alloys containing between 1.90-2.10% Be, I may employ as high as .50% of one or more of the metals Fe, Co and Ni, preferably Co without substantial detriment to the cold working properties of the alloy, but I have found it preferable in most instances to use not over .20% of one or more of these metals Fe, Co and Ni.

As one specific embodiment of this improved alloy composition, an alloy containing Be 1.80%, Co .20%, balance substantially all copper, when cast into a 4" ingot may be rendered substantially free of beta constituent by subjecting the same to only three (3) anneals within the temperature range 1400°-1500° F. for three (3) hour time intervals each in hot working the same from ingot size to a size approximating one inch (1") and will be completely free of the beta constituent if following cold reduction down to about 1/2", the metal is given one more such beta-solutioning annealing. Thereafter, the metal can be cold worked to final size with intermediate half hour anneals to remove work hardening as heretofor customary in the art and on heat treatment to age harden will be found to be uniformly responsive and to have improved physical properties.

In an alloy containing 2% Be, I have found .30% Co to be very effective in producing a final cored structure in the cast ingot with resultant better response to the above described working method. In an alloy containing 1.5% Be, I have found Co as low as .125% to be equally as effective as .20% Co in obtaining a finer cored structure and both alloys evidence substantially identical cold working properties following re-solution of the cast beta constituent in accordance with the present invention.

From the above description of the present invention it is believed apparent that many modifications and departures may be made therein without essential departure therefrom and all such are contemplated as may fall within the scope of the following claims.

What I claim is:

1. The method of working cast beryllium-copper alloys containing 1.5 to 2.10% beryllium, which comprises heating the alloy to a temperature within the range 1400°-1500° F. for a time interval at least sufficient to effect substantial re-solution of the cast beta particles dispersed therethrough, mechanically deforming the alloy on a falling temperature gradient initiating at a temperature within the range 1400°-1500° F. and terminating at about 800° F. to an extent at least effective to disturb the alpha phase surrounding the beta particles, reheating the said alloy to within the range 1400°-1500° F. for a time interval effecting further substantial solution of the said beta particles, and repeating the hot mechanical deformation and reheating operations until the remaining beta particles are insufficient to materially interfere with cold mechanical deformation, then rapidly cooling the said alloy from the final heating to condition the same for cold mechanical deformation.

2. The method of claim 1, wherein following cold mechanical deformation to a size larger than

the desired final size the said alloy is again reheated within the range 1400°-1500° F. for a prolonged time interval effective to obtain re-solution of the remaining beta particles and uniform distribution of the beryllium content of the alloy throughout the mass and then is cooled rapidly to atmospheric temperatures to condition the same for cold mechanical deformation to final size.

3. The method of claim 1, wherein during cold mechanical deformation a plurality of intermediate heat treatments at a temperature within the range 1400°-1500° F. is applied thereto each for a time interval effective to obtain further re-solution of the remaining beta particles and to uniformly distribute the beryllium content of the alloy throughout the mass, each said heating being followed by a rapid cooling to preserve the alpha matrix obtained and to condition the alloy for further cold mechanical deformation.

4. The method of working cast Be-Cu alloys containing Be 1.5-2.10% to obtain a homogeneous structure and uniform distribution of the Be content therein, which comprises subjecting the cast alloy to a plurality of successive and alternate heat treating and hot working operations, each said heat treating operation being for a prolonged time interval at a temperature within the range 1400-1500° F. and each said hot working operations being on a falling temperature gradient initiated at about 1450° F. and terminating at a temperature approximating but not below about 700° F., the extent of deformation effected in each said working operation being at least sufficient to substantially break up the stabilized metal structure formed during the preceding heat treatment operation.

5. The method of working cast Be-Cu alloys containing Be 1.5-2.10% Be to obtain substantially complete re-solution of cast beta particles and substantially uniform distribution of the Be content of the alloy throughout the alloy mass during hot mechanical deformation of the same to condition the alloy for cold mechanical deformation, which comprises first heating the alloy to temperatures within the range 1400-1500° F. for a time interval at least sufficient to obtain Be saturation in the alpha matrix immediately adjacent each beta particle, then hot working the alloy on a falling temperature gradient from a temperature approximating 1450° F. to a temperature approximating but not below about 700° F., the extent thereof being at least sufficient to effect a general breaking up of the Be saturated alpha matrix obtained during the first heating operation and the locating of unsaturated alpha matrix in a position to dissolve more Be from the said beta particles, again reheating as in step one above and again hot working as in step two above, and repeating the said heating and working steps one and two until substantially complete re-solution of the said beta particles has been effected and a homogeneous cold workable structure has been obtained.

6. The method of working cast Be-Cu alloys containing from 1.5-2.10% Be to eliminate therefrom cast beta particles and to produce a substantially homogeneous metal structure therein, which comprises subjecting the cast alloy to an extended heating at temperatures within the range 1400-1500° F., the time interval of said heating being at least sufficient to obtain partial re-solution of the beta particles in the alpha phase surrounding the particles, and following said heating subjecting the alloy to mechanical deformation initially at temperatures approxi-

mating 1450° F. and continuing to a temperature approximating but not lower than about 700° F. the extent of such deformation being at least sufficient to effect a general breaking up of the said alpha phase, reheating the mechanically deformed metal to within the said range 1400-1500° F. for a time interval at least sufficient to obtain further re-solution of the said beta particles and again mechanically deforming at temperatures within the range 1450-700° F., and repeating the said heating and working operations until substantially complete re-solution of the said beta particles is effected.

7. The method of effecting the re-solution of beta particles in cast beryllium-copper alloys containing 1.5 to 2.10% Be, which comprises subjecting the cast alloy to alternate beta solutioning heat treatments and hot working operations, each beta solutioning heat treating operation being at a temperature within the range 1400-1500°

F., for a prolonged time interval to obtain beryllium saturation in the alpha phase adjacent to and surrounding the said beta particles, and each hot working operation initiating at a temperature approximating 1450° F. and being continued on a falling temperature gradient to temperatures approximating but not substantially below about 700° F., the extent of deformation during each working operation being at least sufficient to effect a general breaking up of the said saturated alpha phase to condition the said alloy for the following beta solutioning heat treatment operation and the total number of said alternate operations being at least sufficient to effect substantially complete re-solution of the said beta particles, the uniform distribution of Be and the production of a substantially homogeneous metal structure throughout the mass of the said alloy.